

**1**

3,846,126

**POWDER METALLURGY PRODUCTION OF HIGH PERFORMANCE ALLOYS**

Edward M. Foley, Russiaville, and Dennis G. Dreyer and Herbert E. Rogers, Jr., Kokomo, Ind., assignors to Cabot Corporation

No Drawing. Filed Jan. 15, 1973, Ser. No. 323,502  
Int. Cl. B22f 1/00

U.S. CL. 75—211

12 Claims

**ABSTRACT OF THE DISCLOSURE**

A powder metallurgy process suitable for high performance alloys difficult to compact and/or sinter involves coating the particles with a solid organic binder by dry blending the alloy powder with particles of the binder, mixing the blended particles with a solvent for the binder to produce a plastic mass, consolidating this mass to discrete bodies of an intermediate density, drying the bodies, crushing them and screening the resulting agglomerates, pressing them into green compacts, and sintering those compacts.

Some or all of the starting powder may be ground to smaller particle size. As fine grinding is always accompanied by oxidation of the powder, which is detrimental to sinterability, the grinding is adjusted to produce particles of a limited average size range.

This invention relates to the production by powder metallurgy of articles of hard metal alloys. It is more particularly concerned with production by this method of articles of high performance metal alloys.

The alloys with which this invention is concerned are high performance cobalt-base, nickel-base, and iron-base chromium-containing alloys resistant to wear, heat and corrosion. These alloys either are not workable or are worked with difficulty, and are commonly produced as castings, which may be ground or machined where necessary. Many small articles made from high performance alloys, such as thread guides for textile mills, valve seat inserts, and the like, are tedious and expensive to cast in the quantities that are required. Attempts have been made to produce such articles by powder metallurgical process, such as by slip casting or pressing the articles to shape from fine powders, and then sintering them. However, such processes, which have proved satisfactory and economical for many alloys, have turned out to be difficult and expensive to adapt to alloys as hard as the high performance alloys here concerned.

One difficulty is that of achieving the desired high density in the finished article. It has been generally considered that the powder particles should be of spherical configuration and of a random size distribution over a rather wide range of sizes to provide optimum packing density and so facilitate subsequent densification. In U.S. Pat. 3,639,179 of Steven Reichman et al. of Feb. 1, 1972, Method of Making Large Grain Sized Superalloys, the patentees recommended a size range of about 150 microns to about 10 microns. We have found, however, that a number of high performance alloy powders when compacted in this way can be sintered only in a very narrow range of temperatures, or in some cases not at all.

Experiments have indicated that the sintering of metal powders, in general, can be improved by decreasing the particle size of the powder to —325 mesh or less. If this is done by screening the powder through a fine screen only a fraction of the powder is used, which is not economical. In powder atomized from an alloy melt, which is a type of powder widely used in powder metallurgy, only 25% to 35% of the powder is —325 mesh, for example. We attempted to salvage oversize powder by grinding it to

**2**

finer size and found that sinterable powder of the high performance alloys here concerned could be obtained. In many instances, however, this powder was deficient in coherence under pressure, unless it was ground to a considerably smaller particle size than was necessary for sintering.

In the production of articles from iron powder or the powder of ordinary alloys it is conventional to compress the powder into green compacts, so-called, in the shape of the desired article, and then transfer those compacts to a furnace where they are sintered. Those compacts must keep their shape until the particles are bonded by the sintering operation. The stresses which green compacts must withstand depend, among other considerations, on the shape of the compact and its dimensional tolerances. The bulk density of compacts ranges from about 50% of cast density to about 70% where high compacting pressures are employed. As the density of the sintered article is generally required to be 95% of cast density or better, all compacts shrink from about 25% to as much as 40% or more during sintering. Where the sintered compact must meet close dimensional tolerances the compacts are constrained during sintering. In the manufacture of valve seat inserts which must be made to close inside diameter tolerances, for example, the green compacts are slipped over mandrels and sintered in that position. If the cohesion between the powder particles is insufficient the compacts will crack.

The average particle size required for effective compacting, in the worst case, was found to be less than about 5 microns, and the grinding time necessary for such powder was measured in days. This, of course, considerably increased its cost. Moreover, the greatly increased surface area of the very fine powder and the length of time required for its grinding facilitated oxidation of the powder so that, in spite of all precautions, its oxygen content was much greater than that of atomized powder. This high oxygen content is undesirable for several reasons, one overriding reason being that it narrows the sintering range of the powder. Thus, the sinterable powders were not compatible for many of the alloys, and the compatible powders were, effectively, not sinterable.

It is an object of our invention, therefore, to provide a process of producing articles of high performance alloys by powder metallurgy which economically utilizes atomized powders. Another object is to provide such a process which broadens the range of sintering temperatures. Another object is to provide such a process which tolerates the use of particles of larger screen size than prior known processes. It is still another object to provide a process adaptable to high performance alloys not sinterable by presently known powder metallurgy process. Other objects of our invention will appear from the description thereof which follows.

We have found that compactability of high performance alloy powders is greatly improved by coating the particles with a binder in a way to be described, and that the coarse fraction of the powder can be reduced to a particle size suitable for sintering in a relatively brief grinding operation which does not increase the oxygen content of the powder to unacceptable levels.

Our process to be described is adapted to utilize the full size range of atomized melts of many high performance alloys if maximum density in the resulting article is not desired. It is also adapted to high performance alloys which by conventional processes are unsinterable or marginally sinterable. It comprehends the milling of a relatively coarse fraction of an atomized melt, or the entire product, so as to reduce the particles to a size which is not accompanied by unacceptable oxidation, the dry blending of this powder with a binder, and the mixing of that blend with a solvent for the binder to produce a

plastic mass, the consolidation of this mass to discrete bodies of an intermediate density, the drying and crushing of those bodies and screening of the resulting agglomerates to about —100 mesh size, the pressing of the agglomerates into green compacts which hold their shape, the transfer of those compacts to a furnace, and the sintering of those compacts.

Compositions of a number of alloys for which our process is suitable are listed in the accompanying Table.

COMPOSITIONS OF TYPICAL ALLOYS IN WEIGHT PERCENT

| Alloy  | Alloying elements |      |      |      |       |      |       |      |      |       |       |       |       |
|--------|-------------------|------|------|------|-------|------|-------|------|------|-------|-------|-------|-------|
|        | Co                | Ni   | Si   | Fe   | Mn    | Cr   | Mo    | W    | C    | V     | B     | P     | S     |
| 1..... | Bal.              | *3.0 | *1.0 | *3.0 | *1.0  | 29.0 | ..... | 11.0 | 2.00 | ..... | *1.0  | ..... | ..... |
|        |                   |      |      |      |       | 33.0 | ..... | 14.0 | 2.70 | ..... |       |       |       |
| 2..... | Bal.              | *3.0 | *1.5 | *3.0 | *1.0  | 27.0 | *1.50 | 3.5  | 0.90 | ..... | *1.0  | ..... | ..... |
|        |                   |      |      |      |       | 31.0 | ..... | 5.5  | 1.40 | ..... |       |       |       |
| 3..... | Bal.              | 9.5  | *1.0 | *2.0 | *1.0  | 24.5 | ..... | 7.0  | 0.5  | ..... | *0.04 | *0.04 | ..... |
|        |                   | 11.5 |      |      |       | 26.5 | ..... | 8.0  | 0.55 | ..... |       |       |       |
| 4..... | Bal.              | *3.0 | *1.0 | *5.0 | *1.0  | 24.0 | ..... | 13.0 | 3.00 | ..... | *1.0  | ..... | ..... |
|        |                   |      |      |      |       | 28.0 | ..... | 15.0 | 3.50 | ..... |       |       |       |
| 5..... | Bal.              | *2.5 | *1.0 | *3.0 | *1.0  | 31.0 | ..... | 16.0 | 2.20 | ..... | *1.0  | ..... | ..... |
|        |                   |      |      |      |       | 34.0 | ..... | 19.0 | 2.70 | ..... |       |       |       |
| 6..... | Bal.              | 2.0  | *1.0 | *2.5 | *1.0  | 28.0 | *0.8  | 17.0 | 1.70 | 3.70  | 0.7   | ..... | ..... |
|        |                   |      |      |      |       | 32.0 | ..... | 20.0 | 2.20 | 4.70  | 1.5   | ..... |       |
| 7..... | 9.0               | Bal. | *1.0 | 11.5 | *0.75 | 25.0 | 9.0   | 9.0  | 1.30 | ..... | *1.0  | *0.04 | *0.03 |
|        | 11.0              |      |      | 13.5 |       | 27.0 | 11.0  | 11.0 | 1.50 | ..... |       |       |       |
| 8..... |                   |      | 0.5  | Bal. | *0.5  | 15.5 | 14.5  | 2.90 | 1.65 | ..... |       |       |       |
|        |                   |      | 1.5  |      |       | 18.5 | 17.5  | 3.40 | 2.10 | ..... |       |       |       |

\*Maximum.

NOTE.—Balance includes incidental impurities.

The alloy powder which we employ is preferably produced by the atomization of a melt of the desired composition. This melt is heated to a temperature of 200° F. or so above its fusion temperature in a crucible. Preferably, this melting is carried out in vacuum or under a blanket of inert gas such as argon. The melt is then poured into a preheated refractory tundish which is formed with a small diameter nozzle in the bottom through which the stream of metal flows into an atomizing chamber. The stream emerging from the nozzle is broken up into fine particles by a high-pressure jet of inert gas, or of water, which makes contact with the molten stream just below the nozzle. The particles or droplets are almost instantaneously quenched by the atomizing fluid and fall into a reservoir in the bottom of the atomizing chamber. Only the fraction is used which passes through a 30 mesh screen. These particles are approximately spherical in shape and about 25% to 35% of the particles are —325 mesh. A 325 mesh screen will pass particles the greatest dimension of which is 44 microns.

We prefer to use polyvinyl alcohol as a binder for our powder, but other solid binders which are known to the art are employed. Examples are camphor, methyl alcohol, paradichlorobenzene, chloroacetic acid, naphthalene, benzoic acid, phthalic anhydride, glycerine, Acrowax C, which is a proprietary compound, the ethylene oxide polymers sold as Carbowax, synthetic gums such as acrylamide, and metal stearates. The solvent for the binder must be appropriately chosen. Water is satisfactory for water-soluble binders.

The blending of the powder and binder particles is accomplished in any suitable mixing apparatus. The amount of binder is not critical, and a few percent by weight is sufficient. Extrusion of the plastic or putty-like blend of particles, binder and solvent is the most convenient way of consolidating the plastic mixture into agglomerates, but other methods, such as roll briquetting, may be employed.

The extrusions are then dried, crushed in a roller crusher, hammer mill or the like, and screened. The —100 mesh fraction of crushed extruded binder powder is largely fines. From about 60 to 80% of the particles are —325 mesh with corresponding apparent densities of about 2.0 to 3.3 grams per cc. Both the percentage of fines and the

apparent density of this material are, however, less than those of the milled powder. It is our belief that each particle of powder in the material, as the result of blending and extruding, is coated with a film of binder, and that in the green compacts pressed from this material the powder particles are held together by this binder film.

The agglomerates of powder and binder are pressed in dies or molds of the desired shape under a pressure of about 50 tons per sq. inch, as has been mentioned. The

compacting pressure can be as low as 20 tons per sq. inch or as high as 70 tons per sq. inch, the density of the green compacts being higher at higher compaction pressures. At a compaction pressure of 20 tons per sq. inch, compact density is about 56 to 58% of cast density, and at 70 tons per sq. inch it is 70 to 72% of cast density.

The desired density of the finished article is obtained by sintering the compact in vacuum or reducing atmosphere at a temperature between the solidus temperature and liquidus temperature of the alloy. Sintering can be completed in about an hour, but if the time is extended to two or at most three hours, the temperature can be reduced somewhat without impairing the properties of the article. Compacts properly sintered have densities of 98% or better of cast density.

Our process also contemplates grinding, when necessary, of part or all of the powder particles resulting from the atomization of a melt as above described. We grind relatively coarse atomized powder, such as —30 mesh by ball milling, impact milling, attriting, vibrating milling, or other known process so as to convert it to particles more than 98% of which are —325 mesh and process those particles in the way described above to produce sintered articles having improved properties. The milling vehicle which we prefer to use is methanol, the mill is preferably evacuated to minimize oxidation of the charge, and, in the case of ball milling, the balls charged are made of a wear-resistant alloy of a composition compatible with the product being produced. Milling time ranges from about 8 to 36 hours and the average particle size of the —325 mesh product ranges from about 30 microns to as low as 9 microns, depending on milling conditions. After milling, the charge is dumped from the mill and the powder allowed to settle. The alcohol is decanted and the sludge is vacuum filtered. The powder filter cake is allowed to dry under vacuum or in air, and is then crushed to —60 mesh agglomerates of binderized particles.

Compacts of —30 mesh atomized powder of Alloy No. 7 cannot be sintered. The —325 mesh fraction of this powder, which has an average particle size of about 31 microns, can be sintered, although the temperature range for 95% density is rather narrow. As has been mentioned, however, the —325 mesh fraction of the atomized powder represents only about 25% to 35% of the powder.

The -30 mesh atomized powder milled to an average particle size of about 15 microns can be sintered to 95% density or better within a temperature range of about 25 to 30°. This range is broad enough for commercial operation. The oxygen content of the milled powder is about 0.44%. It is interesting to find that the addition of a relatively minor amount of a fine fraction of the atomized particles to milled powder appreciably impairs its sinterability. In another run a charge of -30 +270 mesh atomized powder of No. 7 alloy was ground in a ball mill for 25 hours to an average particle size of about 10 microns. This material was mixed with -270 mesh atomized powder in amount representing 30% by weight of the aggregate. The average particle size of this aggregate was 23.5 microns. Compacts of the aggregate did not sinter as well as compacts of -30 +270 mesh atomized powder milled in a ball mill for 18 hours to an average particle size of 15 microns. The first mentioned powder had to be sintered at a temperature of 2300° F. for better than an hour to achieve 95% density. Sintering at 2310° F. for an hour resulted in an article density of 98.25%. The second mentioned powder achieved a compact density of 95% after one hour of sintering at 2280° F. and 98% after one hour at 2290° F.

#### EXAMPLE I

The -325 mesh fraction of atomized powder of Alloy No. 3 of the Table was dry blended in a mixer with particles of a binder, preferably -100 mesh polyvinyl alcohol, in amounts of 2% to 3% by weight. The powder particles used had an average particle size of about 30 microns. Then enough warm water was added to form a plastic mixture of the powder and binder. This mixture was then extruded into cylinders or roundels of about two inches long and one-half inch in diameter under pressure sufficient to consolidate the mixture to a density of about 60% of cast density. The roundels were dried, then crushed in a roller crusher, hammer mill, or the like, and the crushed material was screened to -100 mesh. The -100 mesh agglomerates of blended alloy powder particles were formed under pressure of about 50 tons per sq. inch into green compacts of the desired shape, which had sufficient strength to withstand further processing. The green compacts were then sintered for 1 to 3 hours at a temperature of between 2260° F. and 2325° F. The binder volatilized during sintering and the sintered articles had a density of 97% to 99% of cast density.

#### EXAMPLE II

Inert gas atomized powder of Alloy No. 7, a nickel-base alloy, was screened through a 30 mesh screen. One hundred pounds of the screened powder were charged into a 28" long ball mill along with 13 gallons of methanol and about 800 pounds of Haynes Stellite\* Alloy No. 3 balls. The mill was evacuated and run at approximately 80% of critical speed (54 r.p.m.) for 10 hours. The average particle size of the resulting powder was about 17.5 microns. About 98% of the powder was -325 mesh. The powder was removed from the mill, filtered, dried, and dry blended with 2% by weight of -100 mesh polyvinyl alcohol particles, and 1% by weight of Acrowax C, mixed with water to form a putty-like mass, extruded into roundels, dried, crushed, charged into a die, pressed and removed from the die. The coherent green compacts were placed in a sintering furnace and sintered at a temperature between 2210° F. and 2230° F. for a period of time of 1 to 3 hours. The articles resulting had a density of 98% to 99% of cast density and Rockwell C scale hardness of 41 to 44.

#### EXAMPLE III

Inert gas atomized powder of Alloy No. 6, which is a cobalt-base alloy, was milled as is described in Example II except for a time of 36 hours to powder having an aver-

age particle size of 11.5 microns. This powder was then processed as described above, except that 3% polyvinyl alcohol plus 1% Acrowax C constituted the binder, into coherent compacts, which were transferred to a sintering furnace and sintered at a temperature between 2140° F. and 2160° F. The finished articles had a density of 96 to 98% of cast density.

#### EXAMPLE IV

Inert gas atomized particles of Alloy No. 8, which is an iron-base alloy, were screened through a 325 mesh screen. The particles passing through the screen were then mixed with a binder as described in Example I, except that the binder was 3% polyvinyl alcohol, and further processed as there described into green compacts. These compacts held their shape, and were transferred to a sintering furnace and sintered at a temperature between 2150° F. and 2170° F. to articles having a density of 97% of cast density.

#### EXAMPLE V

Inert gas atomized particles of Alloy No. 8 of -30 mesh size were ground in a ball mill for 24 hours to particles of an average particle size of about 9 microns. These particles were then blended with 3% by weight of polyvinyl alcohol particles and 1% by weight of particles of Acrowax C and further processed as is described in Example I into coherent green compacts. Those compacts were sintered at a temperature between 2140° F. and 2170° F. to articles having a density of 97% of cast density.

The vehicle chosen for the ball milling has some effect on the sintering process. While we would prefer to use water, we find that its use results in a measurable increase in the oxygen content of the sintered article and a narrowing of the temperature range for sintering. Where the oxygen content of the alloy is critical or where the sintering range is restricted we use a solvent other than water. In the case of No. 7 alloy, for example, made from powder of about 18 microns average size, the increase in oxygen content of the alloy arising from the use of water as a vehicle is about 0.43%. We prefer to use methanol as a vehicle, which brings about an increase in oxygen content of only about 0.12%. Other organic solvents that may be used as vehicles are ketones, aromatic hydrocarbons and methane series compounds.

On the other hand, the decomposition of organic binders increases the carbon content of the sintered article in amounts between about 0.1% and 0.2%. In Alloy No. 3 and lower carbon high performance alloys known to the art, this increase can be significant, and in such cases we added to the powder small amounts of an oxide of a metal which is reduced by carbon at the sintering temperature. Cobalt oxide is suitable for Alloy No. 3 and is preferred by us. For other alloys, nickel oxide or oxides of other metals compatible with the alloy composition may be used.

Our process is useful in the manufacture from powder of alloys containing a dispersed phase. We have made thereby, alloys consisting of a matrix of Alloy No. 2 having particles of tungsten carbide dispersed therein in amounts from about 25% to about 60% by weight. The tungsten carbide powder is added to the alloy powder and mechanically mixed therewith. The powder mix is then blended with a suitable binder and processed from that point on in the same way as is described in the examples above set out.

In the foregoing description of the process the screen sizes are ASTM screen sizes. Average particle sizes were determined by Sharples Micromerograph.

In the foregoing specification we have described a presently preferred embodiment of this invention, however, it will be understood that this invention can be otherwise embodied within the scope of the following claims.

We claim:

1. The process of making a coherent green compact which holds its shape during sintering from pre-alloyed comminuted powder of a high performance metal alloy which cannot be pressure compacted under pressures up to 70 tons per square inch unless its average particle size is not greater than about 5 microns, comprising processing the alloy powder to an average particle size between about 9 and about 30 microns, mixing the alloy powder with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of pre-alloyed powder particles to provide a substantial fraction of -100 mesh particles at least about half of the -100 mesh fraction of which are -325 mesh, then filling a die of the desired shape with those agglomerates, then compacting the agglomerates in the die under pressure to at least about 50% of the cast density of the alloy so as to produce a coherent green compact, and then removing the compact from the die.

2. The process of claim 1 including the step of sintering the green compact at a temperature between the solidus and liquidus temperature of the alloy.

3. The process of making a coherent green compact which holds its shape during sintering from comminuted powder of a high performance metal alloy which cannot be pressure compacted under pressures up to 70 tons per square inch unless its average particle size is not greater than about 5 microns, comprising processing the alloy powder to an average particle size between about 9 and about 30 microns, mixing the alloy powder with a dry, finely divided organic binder in amounts not greater than about 5% by weight of the alloy powder and a powdered metal oxide which is reduced by carbon at sintering temperatures so as to obtain a uniform dispersion of binder and metal oxide in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction of which are -325 mesh, then filling a die of the desired shape with those agglomerates, then compacting the agglomerates in the die under pressure to at least about 50% of the cast density of the alloy so as to produce a coherent green compact and then removing the compact from the die.

4. The process of making a coherent green compact which holds its shape during sintering from comminuted powder of a high performance metal alloy which cannot be pressure compacted under pressures up to 70 tons per square inch unless its average particle size is not greater than about 5 microns, comprising processing the alloy powder to an average particle size between about 9 and about 30 microns, mixing the alloy powder with a powder of a substance which appears as a dispersed phase in the sintered article and with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction

of which are -325 mesh, then filling a die of the desired shape with those agglomerates, then compacting the agglomerates in the die under pressure to at least about 50% of the cast density of the alloy so as to produce a coherent green compact, and then removing the compact from the die.

5. The process of claim 1 in which the high performance metal alloy is a cobalt-base, nickel-base, or iron-base alloy.

10 6. The process of making a sintered article by means of a coherent green compact which holds its shape during sintering from a comminuted powder of a high performance metal alloy which cannot be pressure compacted under pressures up to 70 tons per square inch unless its average particle size is not greater than about 5 microns, comprising producing an alloy powder by atomizing with a fluid a melt of an alloy consisting of chromium between 24.5% and 26.5%, tungsten between 7.0% and 8.0%, carbon between 0.45% and 0.55%, nickel between 9.5% and 11.5%, silicon up to 1.0%, iron up to 2.0%, manganese up to 1.0%, phosphorous not more than 0.04%, sulfur not more than 0.04%, and the balance cobalt and incidental impurities, screening the atomized powder through a -325 mesh screen, mixing the alloy powder with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction of which are -325 mesh, then filling a die of the desired shape with those agglomerates, then compacting the agglomerates in the die under pressure to at least about 50% of the cast density of the alloy so as to produce a coherent green compact, and then removing the compact from the die.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9

8. The process of making a coherent green compact which holds its shape during sintering from comminuted powder of a high performance metal alloy which cannot be pressure compacted under pressures up to 70 tons per square inch unless its average particle size is not greater than about 5 microns, comprising producing an alloy powder by atomizing an alloy melt with a fluid and in which at least some of the alloy powder is comminuted by grinding it to an average particle size less than about 30 microns but greater than about 9 microns, mixing the 10 alloy powder with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy 15 powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction of which are -325 mesh, then filling a die of the desired shape with those agglomerates, then compacting the agglomerates in the die under pressure to at least about 50% of the cast 20 density of the alloy so as to produce a coherent green compact, and then removing the compact from the die. 25

9. The process of claim 8 in which about 95% or more of the alloy powder mixed with the binder is -325 mesh.

10. The process of making a sintered article by means of a coherent green compact which holds its shape during 30 sintering from a comminuted powder of a high performance alloy which cannot be pressure compacted under pressures up to 70 tons per square inch unless its average particle size is not greater than about 5 microns, comprising producing an alloy which consists of chromium between 28.0% and 32.0%, tungsten between 17.0% and 20.0%, carbon between 1.70% and 2.20%, vanadium between 3.70% and 4.70%, boron between 0.7% and 1.5%, nickel between 2% and 5%, molybdenum up to 0.8%, silicon up to 1.0%, iron up to 2.5%, manganese 40 up to 1% and the balance cobalt and incidental impurities, by comminuting the alloy powder to an average particle size of about 12 microns or less mixing the alloy powder with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction of which are -325 mesh, then filling a die of the desired shape with those agglomerates, then compacting the agglomerates in the die under pressure to at least about 50% of the cast 45 density of the alloy so as to produce a coherent green compact, and then removing the compact from the die, and then sintering the alloy at a temperature between about 2140° F. and about 2160° F.

11. The process of making a sintered article by means of a coherent green compact which holds its shape during sintering formed from a comminuted powder of a high performance alloy which cannot be pressure compacted under pressures up to 70 tons per square inch unless its average particle size is not greater than about 5 microns, comprising producing an alloy which consists of chromium between 25.0% and 27.0%, molybdenum between 9.0% and 11.0%, tungsten between 9.0% and 11.0%, carbon 50

between 1.30% and 1.5%, iron between 11.5% and 13.5%, phosphorus not more than 0.04%, sulfur not more than 0.3%, manganese up to 0.75%, silicon up to 1.0%, boron up to 1.0%, cobalt between 9.0% and 11.0% and the balance nickel and incidental impurities, by comminuting the alloy powder to an average particle size of about 18 microns or less, mixing the alloy powder with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction of which are -325 mesh, then filling a die of the desired shape with those agglomerates, then compacting the agglomerates in the die under pressure to at least about 50% of the cast density of the alloy so as to produce a coherent green compact, and then removing the compact from the die and then sintering the alloy at a temperature between about 2210° F. and about 2230° F.

12. The process of making a sintered article by means of a coherent green compact which holds its shape during sintering formed from a comminuted powder of a high performance alloy which cannot be pressure compacted under pressures up to 70 tons per square inch unless its average particle size is not greater than about 5 microns, comprising producing an alloy which consists of chromium between 15.5% and 18.5%, molybdenum between 14.5% and 17.5%, carbon between 2.90% and 3.40%, vanadium between 1.65% and 2.10%, silicon between 0.5% and 1.5%, manganese up to 0.5% and the balance iron and incidental impurities, by comminuting the alloy powder to an average particle size of about 12 microns or less, mixing the alloy powder with a dry, finely divided organic binder in amounts not greater than about 5% by weight of the alloy powder so as to obtain a uniform dispersion of binder in the alloy powder, then adding a solvent for the binder in amount sufficient to form a plastic mixture with the alloy powder and binder, then consolidating the plastic mixture to a bulk density intermediate that of the powder and that of the cast alloy, then drying the consolidated mixture to evaporate the solvent, then crushing the consolidated mixture to discrete agglomerates of alloy powder particles at least about half of the -100 mesh fraction of which are -325 mesh, then filling a die of the desired shape with those agglomerates, then compacting the agglomerates in the die under pressure to at least 50% of the cast density of the alloy so as to produce a coherent green compact, and then removing the compact from the die, and then sintering the alloy at a temperature between about 2140° F. and about 2170° F.

#### References Cited

##### UNITED STATES PATENTS

|           |         |                 |       |        |
|-----------|---------|-----------------|-------|--------|
| 2,857,270 | 10/1958 | Brundin         | ----- | 75—213 |
| 3,639,179 | 2/1972  | Reichman et al. | ----- | 75—171 |
| 3,615,381 | 10/1971 | Hammond         | ----- | 75—213 |
| 3,671,230 | 6/1972  | Smythe et al.   | ----- | 75—213 |

65 65 CARL D. QUARFORTH, Primary Examiner

B. HUNT, Assistant Examiner

U.S. Cl. X.R.

70 75—200, 213, 221

UNITED STATES PATENT OFFICE  
CERTIFICATE OF CORRECTION

Patent No. 3,846,126

Dated November 5, 1974

Inventor(s) Edward M. Foley et al.

It is certified that error appears in the above-identified patent and that said Letters Patent are hereby corrected as shown below:

Column 1, line 66, "particl" should read --particle--.

In the Table, Columns 3 and 4, Alloy 3, under element C, "0..5" should read --0.45--.

Column 10, Claim 11, line 3, "0.3%" should read --0.03%--.

Signed and sealed this 14th day of January 1975.

(SEAL)

Attest:

McCOY M. GIBSON JR.  
Attesting Officer

C. MARSHALL DANN  
Commissioner of Patents